

July 14, 1953

N. S. MORETON

2,645,745

PERMANENT MAGNET ASSEMBLY

Filed April 17, 1952

3 Sheets-Sheet 1

FIG. 1



FIG. 4



FIG. 2



FIG. 5



FIG. 3



FIG. 6



FIG. 7



FIG. 25

FIG. 8



Witnesses:

Roland MacIntyre  
John L. Stern

INVENTOR.  
Neal S. Moreton,

BY  
Ralph Hammars  
His Attorney.

July 14, 1953

N. S. MORETON

2,645,745

PERMANENT MAGNET ASSEMBLY

Filed April 17, 1952

3 Sheets-Sheet 2



Witnesses:

Roland Mac Intyre  
John A. Stevens

INVENTOR.  
Neal S. Moreton,  
BY  
Ralph Hammars  
His Attorney.

July 14, 1953

N. S. MORETON

2,645,745

PERMANENT MAGNET ASSEMBLY

Filed April 17, 1952

3 Sheets-Sheet 3



FIG. 24



Witnesses :

Roland MacIntyre  
John L. Sturr

INVENTOR.  
Neal S. Moreton,  
BY  
Ralph H. Hammars  
His Attorney.

## UNITED STATES PATENT OFFICE

2,645,745

## PERMANENT MAGNET ASSEMBLY

Neal S. Moreton, Staten Island, N. Y.

Application April 17, 1952, Serial No. 282,844

2 Claims. (Cl. 317—161)

1

This application is a continuation-in-part of application Serial No. 35,167, filed June 25, 1948, now abandoned.

The high strength permanent magnets of the aluminum nickel cobalt type usually require pole shoes and some form of supporting frame which has been difficult to provide due to the hardness and brittleness of the magnet material. This invention is intended to cast the supporting frame uniting the magnets and associated pole shoes with a non-magnetic material having the properties of setting in place and wetting or bonding to the magnets and pole shoes. This construction is particularly advantageous in magnetic separators for removing tramp iron. Another feature is a magnetic cement which sets up without the porosity accompanying evaporation of solvent, securing the pole shoes to the magnets.

In a preferred form, the binding ingredient for the cast frame and for the cement is a solventless varnish. This varnish or resin is a fluid which sets to the solid state without the evolution of volatile matter at a rate determined by a catalyst. Further objects and advantages appear in the specification and claims.

In the accompanying drawings, Fig. 1 is a perspective of a pulley type magnetic separator; Fig. 2 is a perspective of a plate type magnetic separator associated with a conveyor belt; Fig. 3 is a perspective of a chute type magnetic separator; Figs. 4, 5, and 6 are views of permanent magnets forming part of the pulley and plate type magnetic separators; Figs. 7 and 8 are perspectives of a hinged magnetic separator plate using the permanent magnet of Fig. 5; Fig. 9 is a top plan view of a magnetic separator plate using the permanent magnet of Fig. 6; Fig. 10 is a section on line *a*—*a* of Fig. 9; Fig. 11 is a section on line *b*—*b* of Fig. 9; Fig. 12 is a top plan view of another magnetic separator plate; Fig. 13 is a section on line *c*—*c* of Fig. 12; and Fig. 14 is a section on line *d*—*d* of Fig. 12; Fig. 15 is a top plan view of another magnetic separator plate; Fig. 16 is a section on line *g*—*g* of Fig. 15; Fig. 17 is a section on line *f*—*f* of Fig. 15; Fig. 18 is an end view of the Fig. 15 plate; Fig. 19 is a side view, partly in section on line *h*—*h* of Fig. 20 of a solid hub magnetic separator; Fig. 20 is an end view, partly in section, on line *k*—*k* of Fig. 19; Figs. 21 and 22 are fragmentary views illustrating the attachment of the pole shoes by a magnetic cement; Fig. 23 is a side view, partly in section, on line *m*—*m* of Fig. 24 of a hollow hub magnetic separator pulley; Fig. 24 is an end view,

2

partly in section, on line *n*—*n* of Fig. 23; and Fig. 25 is a perspective of another magnetic separator plate.

Referring to the drawing, Fig. 1 shows a typical pulley type magnetic separator having a pulley 1 over which runs a conveyor belt 3 carrying non-magnetic material 2 such as textile fibers, grain, coal, or liquids from which it is desired to remove tramp iron or particles of ferrous or magnetic material indicated generally by the reference numeral 3. The pulley contains permanent magnets 4 which cause the magnetic material to be held against the conveyor belt until forcibly removed as the belt runs off the underside of the pulley. In Fig. 2, the conveyor belt runs over a conventional pulley 7, moving the non-magnetic material under plate type magnet 9 having permanent magnets 5 which attract the magnetic material. In Fig. 3, the non-magnetic material is fed through the chute 23 having a hinged plate 10 in its bottom wall carrying permanent magnets 6 which pick up the magnetic material. The hinging of the plate 10 permits convenient removal of the adhering magnetic particles when the chute is not in use. Figs. 1, 2, and 3 indicate typical magnetic separator installations.

In each of these separators, permanent magnets of high strength material, such as "Alnico" 30 are used. In order to obtain the most effective separation, these magnets require soft iron pole shoes to obtain the proper magnetic flux distribution. These magnets also require a non-magnetic supporting frame which has been difficult to provide due to the hardness and brittleness of the permanent magnet material.

In the present invention, the supporting frame for the permanent magnets, the associated pole shoes, and other component parts is provided by a non-magnetic compound containing a solventless varnish or resin, a catalyst and a filler such as talc, glass fiber or other textile fibers or fillers. The purpose of the filler is to increase the strength or other mechanical properties of the compound. One type of solventless varnish or resin employed in this compound, for example, is an unsaturated polyester of the addition polymerization type. Another type of solventless varnish or resin employed in the compound used in this invention, for example, is a condensation polymerization type having the property of curing to its final state without the evolution of volatile matter. The unsaturated polyester (addition polymerization type) of solventless varnish or resin also has the property of setting up

from the liquid to the solid or cured state without the evolution of volatile matter. These varnishes produce a dense non-porous structure and also have the property of wetting metal and producing a strong metal to resin bond.

In order to increase the effectiveness of the magnetic pull of the magnets, the pole shoes are preferably attached to the magnets by a cement containing powdered magnet material. Such a cement may contain a solventless varnish, a catalyst, and powdered "Alnico." A similar result may be reached by a mixture of powdered metals corresponding to the analysis of "Alnico" or other suitable permanent magnet material. The solventless varnish ingredient in the cement may be an unsaturated polyester of the addition polymerization type or the condensation polymerization type which cures without the evolution of volatile matter. This cement sets in place and forms a good bond between each pole face of the permanent magnet and its corresponding pole shoe and in addition to eliminating the gap between the pole faces of the magnet and their corresponding pole shoes, it also prevents the casting compound of the frame structure from flowing in between the magnet pole faces and their corresponding pole shoes.

The magnetic cement, in effect, becomes a part of the permanent magnet, thereby improving the effectiveness of the magnet assembly even though the pole surfaces of the magnet are not carefully ground to fit the pole shoes.

The following is an example of the casting compound for the supporting frame:

|                                                                          | Parts by weight |
|--------------------------------------------------------------------------|-----------------|
| Solventless varnish (Unsaturated polyester addition polymerization type) | 125.0           |
| Tertiary butyl perbenzoate or benzoyl peroxide (Catalyst)                | 1.3             |
| Filler                                                                   | 60.0            |

An alternate example of casting compound:

|                                                                                                        | Parts by weight |
|--------------------------------------------------------------------------------------------------------|-----------------|
| Solventless varnish (Condensation polymerization type that cures without evolution of volatile matter) | 110.0           |
| Benzoyl dimethylamine (Catalyst)                                                                       | 11.0            |
| Filler                                                                                                 | 60.0            |

An example of the magnetic cement employed:

|                                                                          | Parts by weight |
|--------------------------------------------------------------------------|-----------------|
| Solventless varnish (Unsaturated polyester addition polymerization type) | 14.85           |
| Tertiary butyl perbenzoate or benzoyl peroxide (Catalyst)                | 0.15            |
| Powdered "Alnico" magnet material                                        | 85.00           |

An alternate example of magnetic cement:

|                                                                                                        | Parts by weight |
|--------------------------------------------------------------------------------------------------------|-----------------|
| Solventless varnish (Condensation polymerization type that cures without evolution of volatile matter) | 13.65           |
| Benzoyl dimethylamine (Catalyst)                                                                       | 1.36            |
| Powdered "Alnico" magnet material                                                                      | 85.00           |

The powdered "Alnico" magnet material in either of the two examples of cement given may be substituted by the following:

|                   | Parts by weight |
|-------------------|-----------------|
| Powdered aluminum | 6.08            |
| Powdered cobalt   | 20.04           |
| Powdered nickel   | 11.09           |
| Powdered copper   | 2.55            |
| Powdered iron     | 45.24           |

In these combinations, the catalyst is for the purpose of accelerating the setting up of the resin. Other catalysts may be used and the amount may be varied to suit conditions. The amount and character of the filler in the casting compound and the powdered magnetic material in the cement are likewise subject to considerable variation. In constructing the magnetic separator

plates, the pole shoes which may be strips of soft iron (steel) 11 and 18 may be placed in a mold with the outer or working faces down. Magnetic cement may be applied on the upper faces of the strips and the permanent magnets placed on the strips and worked around so as to squeeze any excess magnetic cement from between the magnet and the associated pole shoes. The magnetic cement will usually form a bead 17 at the sides of the magnet, as indicated in Figs. 21 and 22. After the magnets are located on the pole shoes, other components may be added and the casting compound is poured into the mold where it sets up in situ, when converted to its cured or final state by cold setting or by the application of heat.

In the structure shown in Figs. 7 and 8 where the cast material extends beyond the edges of the pole shoes and must have sufficient strength at its edges to carry the weight, it may be desirable to lay fibrous reinforcing material into the mold at the points where reinforcement is desired. In constructions such as shown in Figs. 17 and 18, the casting compound merely embeds the central parts of the pole shoes 18. With this construction, a greater thickness is necessary at the center to provide sufficient mechanical strength.

In the pulley type separators shown in Figs. 19 and 20, the pulley shaft 15 has non-magnetic end flanges 16 fixed thereto. Between the flanges are fixed spaced axially extending pole shoes 13 which have curved surfaces corresponding to the desired outer surface of the pulley. The magnets 4 have curved poles which bridge the under sides of the pole shoes 13. The permanent magnets will ordinarily be cemented to the pole shoes before the pole shoes are mounted on the flanges 16. After assembly, a sheet is wrapped around the pole shoes 13 to close the spaces between the pole shoes and casting compound 14 poured into the interior through an opening x in one of the flanges 16. After setting, the wrapping sheet is removed and a smooth pulley surface is obtained in which the casting compound 14 is substantially flush with, or a continuation of the outer working surfaces of the pole shoes 13. In a larger diameter pulley type separator, in order to cut down the amount of casting material, and flanges 20 mounted on a shaft 21, are provided with inwardly extending flanges 25 which carry a cylinder 22 spaced slightly inward from the permanent magnets 4. In this construction, the opening x through which the casting compound is poured into the mold cavity is located in one of the end flanges 20 between the cylinder 22 and the outer surface of the pulley.

In all these constructions, the casting compound flows around the poles of the magnet and the adjacent faces of the pole shoes and in the space between the spaced pole shoes and provides a smooth surface which is substantially flush with the outer exposed working surfaces of the pole shoes. The characteristics of this casting compound is such that a frame structure of great strength and rigidity may be formed. It is also odorless, substantially chemically inert in that it is resistant to alkalies, acid, heat, cold, and corrosion. It also adheres or bonds well to metal inserts and other component parts of the structure. The absence of crevices in the working face in which the material being treated (material in process) can lodge, provides a permanent magnet structure which in actual practice keeps clean, except for the tramp iron, and therefore can operate effectively for longer periods. This

is an advantage over and above the increased magnetic pull.

What is claimed as new is:

1. A magnet assembly for magnetic separators comprising a pair of spaced soft iron pole shoes, each shoe having an exposed working face, a U-shaped permanent magnet having a pole adjacent the face of each pole shoe opposite its working face, there being a gap between each pole and pole shoe, a magnetic cement in the gaps forming an adherent mechanical connection between the poles and pole shoes, said cement comprising a mixture of finely divided material having the characteristics of permanent magnets and a solventless varnish of the unsaturated polyester type set up by addition polymerization without the evolution of volatile matter, said cement being set up in situ in each gap and a non-magnetic frame for the magnetic assembly comprising a solventless varnish of the unsaturated polyester type set up by addition polymerization without the evolution of volatile matter cast and set up in situ around the poles of the magnet and the adjacent faces of the pole shoes and in the space between the spaced pole shoes.

2. A magnet assembly for magnetic separators comprising a pair of soft iron pole shoes having spaced generally parallel inner edges, each shoe

having an exposed working face, a permanent magnet bridging the space between the inner edges of the pole shoes and having a pole adjacent the face of each shoe opposite its working face, there being a gap between each pole and pole shoe, a magnetic cement in the gaps forming an adherent mechanical connection between the poles and pole shoes, said cement comprising a mixture of finely divided aluminum nickel cobalt type permanent magnet material and a solventless varnish set up in situ without the evolution of volatile matter, and a non-magnetic supporting frame for the magnet assembly comprising solventless varnish cast in situ without the evolution of volatile matter flush with the exposed working faces of the pole shoes and around the reverse faces of the pole shoes and the adjacent poles of the magnet to provide a rigid structure having a smooth surface even with the exposed working faces of the pole shoes.

NEAL S. MORETON.

References Cited in the file of this patent

UNITED STATES PATENTS

| Number    | Name     | Date         |
|-----------|----------|--------------|
| 1,834,898 | Boyajian | Dec. 1, 1931 |